

July 17, 1923.

1,462,074

W. O. SNELLING

DETONATOR

Filed June 14, 1919

*Fig. 1.*



*Fig. 2.*



*Inventor:*  
Walter O. Snelling  
*by his Attorney:*  
Howson & Howson

## UNITED STATES PATENT OFFICE.

WALTER O. SNELLING, OF ALLENTOWN, PENNSYLVANIA, ASSIGNOR TO TROJAN POWDER COMPANY, OF NEW YORK, N. Y., A CORPORATION OF NEW YORK.

## DETONATOR.

Application filed June 14, 1919. Serial No. 304,215.

To all whom it may concern:

Be it known that I, WALTER O. SNELLING, a citizen of the United States, and resident of Allentown, Lehigh County, Pennsylvania, have invented certain Improvements in Detonators, of which the following is a specification.

My invention relates to improvements in initial detonating agents, and refers more particularly to the preparation of detonating caps and electric detonators having a nitrostarch explosive base.

Hitherto, the employment of nitrostarch as the explosive base in detonators and the like has been unsuccessful, owing to the fact that the nitrostarch, when completely confined in a detonating capsule, rapidly undergoes decomposition, the first traces of decomposition products acting as catalysts, and rapidly bringing about decomposition of the remaining material. Such detonators have been incapable of withstanding storage conditions, and actual tests have shown that a temperature of 100 degrees C. for from five to eight hours is usually sufficient to bring about explosion.

I have discovered that detonating caps and electric detonators can be made from nitrostarch, and be capable of meeting successfully the most stringent storage conditions, and these detonators have actually withstood temperatures higher than the average temperature prevailing in magazines, even in the tropics, for many months without diminution in strength or alteration in stability. To produce this result I employ nitrostarch which is free from decomposable lower nitric acid esters of starch, a method of preparing such nitrostarch being fully set forth and described in my copending application Serial No. 268,498, filed December 27th, 1918, and to secure more satisfactory brisance and stability, I may admix with such nitrostarch a suitable oxidizing agent, such as potassium chlorate or ammonium perchlorate, and a stabilizing agent such as diphenylamine, urea, or dicyandiamid. This nitrostarch I employ as my detonator base, and in connection therewith I prefer to use a priming charge of a suitable primary detonating agent such as mercury fulminate, lead azid, or the like.

As illustrating a detonator made in accordance with my invention, I may em-

ploy a detonator cap of the type illustrated in the accompanying drawings, in which:

Figure 1 is a vertical section of a detonator cap made in accordance with my invention; and

Figure 2 is an enlarged perspective of the inner capsule.

With reference to the drawings, the cap comprises an outer shell or capsule, 1, closed at one end, which receives the base or main charge, and an inner capsule, 2, disposed within the outer capsule, 1, and containing a suitable priming charge, both inner and outer capsules being made of copper, nickel, or other suitable material. The base or main charge comprises my nitrostarch free from decomposable lower nitric esters of starch, mixed with suitable proportions of an oxidizing agent and a stabilizing agent if desired, and the priming charge preferably comprises mercury fulminate, lead azid, or other primary detonating agent. To make a detonator cap having the same strength as a detonating cap of mercury fulminate of what is called "No. 6" grade, and corresponding to a charge of one gram of mercury fulminate, I prefer to employ an outer capsule of copper, 5.60 mm. in inside diameter, and 38 mm. in length. As an inner capsule I prefer to employ a capsule 5.50 mm. in outside diameter and 9 mm. in length. As my priming charge I may employ .4 g. of a mixture of 80 parts of mercury fulminate and 20 parts of potassium chloride, and as my main charge I may employ .5 g. of a mixture consisting of 80% of nitrostarch of approximately 13% nitrogen, and free from decomposable lower nitric acid esters of starch, 15% of ammonium perchlorate, and 5% of diphenylamine. I press the charge as indicated into my detonating capsule under a pressure of 90 kg., and under these circumstances I obtain detonating caps which are both stable and satisfactory, will withstand a temperature of 100° C. for several months without exploding, and which will withstand a temperature higher than the average temperature prevailing in magazines, even in the tropics, for many months without diminution in strength nor alteration in stability.

I have found that the best results are obtained when from 70% to 90% of nitrostarch

is used with from 10% to 25% of potassium chlorate or ammonium perchlorate and 1% to 10% of diphenylamine, urea, or dicyandiamid, but I do not wish to be limited to 5 any specific proportions in which the various elements of the explosives may be mixed, since it is obvious that wide latitude in this respect is allowable with minor changes in the strength and explosive character of the 10 detonator only, and with no departure from the essential features of the invention. Nor do I wish to be limited to the particular method of preparing nitrostarch free from decomposable lower nitric acid esters of 15 starch herein mentioned, since I have discovered that nitrostarch made by any process, if free from decomposable lower nitric acid esters of starch, is suitable for use in making stable and satisfactory detonators.

20. I claim:

1. A detonator comprising an initial prim-

ing charge and a main charge comprising nitrostarch.

2. A detonator comprising an initial priming charge comprising mercury fulminate, 25 and a main charge comprising nitrostarch.

3. A detonator comprising an initial priming charge, and a main charge comprising nitrostarch and an oxidizing agent.

4. A detonator comprising an initial priming charge, and a main charge comprising nitrostarch and potassium chlorate. 30

5. A detonator comprising an initial priming charge, and a main charge comprising nitrostarch, an oxidizing agent, and a stabilizing agent. 35

6. A detonator comprising an initial priming charge, and a main charge comprising nitro-starch, potassium chlorate, and diphenylamine.

WALTER O. SNELLING.